

Jan. 31, 1933.

S. RUBEN

1,896,043

INSULATED WIRE AND PROCESS THEREFOR

Filed Dec. 3, 1930

*Fig. 1*



*Samuel Ruben*  
INVENTOR

BY *Karl Goldstein*  
ATTORNEY

## UNITED STATES PATENT OFFICE

SAMUEL RUBEN, OF NEW ROCHELLE, NEW YORK, ASSIGNOR TO VEGA MANUFACTURING CORPORATION, OF WILMINGTON, DELAWARE, A CORPORATION OF DELAWARE

## INSULATED WIRE AND PROCESS THEREFOR

Application filed December 3, 1930. Serial No. 499,845.

This invention relates to an improved type of insulated wire and to a method of making the same.

An object of the invention is to produce 5 a wire having a flexible refractory insulation.

A further object is the provision of a wire having a closely applied flexible insulating coating containing refractory inorganic 10 material unaffected by high temperatures.

Other objects will be apparent from the description of the invention and from the drawing in which is shown an insulated wire made in accordance with the invention.

15 I have found that in order to properly coat a wire with an insulating material having the desired characteristics, it is desirable also to have, (1) a flexible binder of the resinous type to give a proper bond at low temperature and (2) a further binder, which material is to be effective at high temperatures. This second binder must be of the inorganic type such as boric acid or lead borate and it serves 20 two important purposes: one, it binds the refractory and insulating material at high temperature; two, it prevents scaling and surface oxidation.

The coating may consist of a refractory 25 oxide, a gum or resinous binder and a borate or other inorganic relatively high temperature binding agent.

The insulating or refractory material used in the coating of this invention may consist of one or more of the refractory oxides, for 30 example, chromium sesqui-oxide, aluminum oxide, magnesium oxide, beryllium oxide, titanium oxide, zirconium oxide or combinations of these, the chromium oxide, however, being preferred. I may also use other compounds containing the silicates, such as beryl or mica. The material used should be ground to as fine a state as possible.

As a flexible binder of the resinous type I prefer to use shellac and Venice turpentine 45 in a volatile solvent such as alcohol or amyl acetate. For the relatively high temperature binder I prefer to use boric acid.

In the coating of some wires, notably copper, in order to have the insulating coating 50 adhere to the copper and prevent surface

oxidation effects, I have found that it is desirable to preliminarily coat the wire with a coating that is integral with the base and preferably fused thereon, such as a solvent oxide coating. For this purpose I have 55 found that a fused on layer of antimony oxide is especially suited; or the wire may also be treated by passing it through a borate solution and heating it, whereupon (if copper) it acquires a hard red fused surface. 60

In a typical coating mixture I use 200 65 grams of chromium sesqui-oxide, 100 grams of boric acid, 100 grams flake shellac, 100 grams of Venice turpentine and 450 cc. alcohol. The shellac is first dissolved in the 70 alcohol after which the chromium sesqui-oxide and boric acid are added. This mixture is milled until the various materials are thoroughly ground after which the Venice turpentine is added and thoroughly admixed. 75 The solution is then ready to be used. The figures given for the composition of the coating may be varied by increasing or decreasing the respective amount of its constituent elements according to the nature of the coating desired; it being recognized that in some cases less flexibility and greater insulation or vice versa may be desired.

The process used is that of a continuous 80 coating whereby the wire is passed through a mixture of antimony oxide in alcohol, then into a furnace which dries the mixture and melts it. The fused antimony oxide flows over the surface of the wire and when cool presents a tough integral layer of minute 85 thickness. The wire then passes through cups containing the insulating compound, being heated and baked, in furnaces located between the cups, to a temperature just below that at which the coating darkens. During 90 the heating, the inorganic binder of boric acid melts and binds the refractory oxide crystals, a great part of the organic materials being baked off. The thickness of the coating is regulated by the consistency of the solution, the speed with which the wire passes through the coating cups, the number of cups used, the temperature of the furnace and the size of the wire. Even though the wire may be heated to a point where the organic bind- 100

er is disengaged no harm results due to the presence of the inorganic binder, boric acid. The use of this borate in the coating also dispenses with the necessity of a flux in soldering the wire, particularly when copper wire is coated.

While the initial process of fusing on a layer of antimony oxide is desirable, it is not necessary, and fairly satisfactory wire can 10 be produced without this initial step.

In some cases in order to further moisture-proof the wire and to increase its flexibility a thin finish coating of lacquer or enamel may be applied.

15 In the drawing, the insulated wire (1) is composed of copper base (2) having formed thereon an integral oxide coating (3) upon which the insulation (4) has been coated. Covering this insulation is waterproof lacquer coating (5).

I claim:

1. An insulated wire comprising a metal base, an oxide coating formed integral with said base, and a coating of finely divided insulating material upon the first coating and held in position by a binder effective at low temperatures and a second binder capable of standing a red heat.

2. An insulated wire comprising a metal 30 base, a fused layer of antimony oxide upon said wire, and a coating of finely divided insulating material held together and upon said wire by an organic binder effective at relatively low temperatures and an inorganic 35 binder capable of standing a red heat.

3. An insulated wire comprising a metal base, a layer of fused oxide integrally formed upon said wire, and a coating of finely divided insulating material held together and 40 upon said layer by an organic binder and an inorganic binder composed of boric acid.

4. In an insulated wire a copper base, a fused layer of oxide formed integrally with said base, and a coating of finely divided insulating material upon said layer and held together by an organic binder composed of shellac, Venice turpentine, and alcohol and a second binder of boric acid.

5. An insulated wire comprising a metal 50 base, a fused layer of antimony oxide upon said base and formed integrally therewith, and a coating of finely divided insulating material held together and upon said base by an organic binder and a second binder capable 55 of standing the temperature of red heat, and a coating of waterproof material upon said insulating coating.

6. An insulated wire comprising a copper base, a layer of a fused oxide formed integral- 60 ly upon said base, a coating of finely divided chromium sesqui-oxide upon said layer and held together and upon said layer by an organic binder and an inorganic binder capable of standing temperatures at red heat, and 65 a surface layer of a moisture-proof material upon said coating.

7. The process of insulating a wire which comprises dissolving an oxide in alcohol, coating the wire with a layer of the dissolved oxide, heating the wire so as to fuse the oxide integrally with the wire, mixing the insulating oxide with an organic binder and with an inorganic binder capable of standing a tem- 70 perature of red heat, successively coating said mixture upon the wire to form a layer thereon and heating said wire so as to dry the 75 layer, until the desired thickness is reached, and coating said second layer with a layer of moisture-proof material.

8. The process of insulating a wire which comprises coating the wire with antimony 80 oxide dissolved in alcohol, heating the wire so as to fuse said oxide to the wire, mixing an insulating oxide with Venice turpentine, shellac, alcohol, and boric acid, applying a plurality of coatings of said mixture upon 85 the fused oxide layer on the wire, heating said mixture after each coating so as to dry it upon the wire, and applying a surface coating of waterproof material to the last coating.

Signed at New Rochelle in the county of Westchester and State of New York this 2nd day of December A. D. 1930.

SAMUEL RUBEN.

90

95

100

105

110

115

120

125

130